

# UNITED STATES PATENT OFFICE.

RENÉ BOTSON, OF AUDERGHEM-BRUSSELS, BELGIUM.

## TREATMENT OF HIDES AND SKINS PRELIMINARY TO TANNING.

No Drawing. Application filed May 21, 1927, Serial No. 193,381, and in Belgium June 2, 1926.

The present invention relates to the treatment of hides and skins preliminary to tanning and has for its object the neutralization of same after they have been unhaired and 5 before their introduction in the tanning bath.

Chemical processes for unhauling hides and skins are well known, as for instance using a solution of steam refined sodium sulphide and caustic alkali with water. It is 10 often preferred to have the hides and skins, after depilation, completely neutralized and specially freed from any particle of lime they may contain.

Up to now, weak acid baths were generally used for the elimination of lime out of unhaired hides and skins, but it has been found that a weak acid bath containing a proportion of nitro-benzol produces a particularly efficient result, so that all mineral im- 15

20 purities will be entirely eliminated.

Following the nature of the hide, the novel treatment will, for instance, comprise a soak-

ing, during 2 to 24 hours, in a bath constituted with acetic acid containing in solution  $\frac{1}{10}\%$  of nitro-benzol, the bath being formed 25 with one part of acid and two thousand parts of water. In these conditions complete neutralization of the hides and skins will be operated and they will be prepared to be 30 tanned in the best conditions with specified tanning materials.

I claim:

1. The treatment of unhaired hides and skins preliminary to tanning consisting in soaking them in weak acid baths containing 35 a very small proportion of nitro-benzol.

2. Neutralizing bath for unhaired hides and skins constituted with one part of acetic acid and two thousand parts of water, the acid containing one part per thousand of 40 nitro-benzol.

In testimony whereof I signed hereunto my name.

RENÉ BOTSON.